

## UNITED STATES PATENT OFFICE

2,339,821

## MANUFACTURE OF WROUGHT IRON

Edward B. Story, Bethel Township, Allegheny County, Pa., assignor to A. M. Byers Company, Pittsburgh, Pa., a corporation of Pennsylvania

No Drawing. Application May 15, 1942,  
Serial No. 443,141

5 Claims. (Cl. 75—47)

This invention relates to manufacture of wrought iron by the Aston process. It relates more particularly to the discovery of certain factors contributing to the production by the Aston process of wrought iron of superior quality.

In the manufacture of wrought iron by the Aston process molten refined ferrous material is admixed with molten iron oxide silicate slag to form a sponge ball in the presence of an excess of slag, the ball is separated from the excess slag which does not become incorporated in the ball and the thus separated ball is compressed to expel a portion of the slag contained therein whereby to form a wrought iron mass or bloom which may be rolled or otherwise worked. Preferably the molten refined ferrous material is poured into a bath of molten slag, the ferrous material passing downwardly through the slag bath and being disintegrated during such passage and forming at the bottom of the receptacle in which the slag is contained a welded spongy mass of metal with slag inclusions commonly referred to as a "ball."

For production of wrought iron of high quality the slag included in the ball should be squeezed out to the greatest possible extent. The compression or squeezing of the ball may be accomplished in any suitable apparatus, a hydraulic press being preferred. It is important that the ball as delivered to the press be at as high a temperature as possible consistent with good practice in other respects as the higher the temperature of the ball as delivered to the press the more included slag will be squeezed out. There is a practical limit to the squeezing or compressing pressure which can be applied to the ball and the results which can be obtained by increase of pressure for a ball of given temperature and it is not practicable to endeavor to make up for relatively low temperature of the ball by the application of relatively high pressure in the press to thereby attempt to squeeze out as much slag as would normally be squeezed out of a ball of desirably high temperature.

I have found that the shape of the ball formed in the slag receptacle has a direct bearing upon the results obtained in the press. The ball should approach as nearly as practicable the shape of a sphere for theoretically best results, although due to the conditions obtaining in making of the ball it is not possible to obtain this maximum theoretical desideratum. Superior results are obtained if the greatest transverse dimension of the ball is not greater than twice its thickness. Preferably the ball approaches cir-

cular shape in transverse cross section and its transverse dimension is roughly equal to its thickness. Depending upon the shape of the receptacle the ball may have more or less flat side faces and a more or less flat bottom, and in such case it is desirable that its shape approach that of a cube with outwardly curved faces and curved edges and corners.

The primary consideration with respect to the shape of the ball is that its surface should be as limited as practicable relatively to its volume. A sphere has the least surface per unit of volume of any solid. The smaller the exposed surface of the ball relatively to its volume the less will be the heat loss between the time the ball is separated from the excess slag and the time it is squeezed in the press. Also the smaller the exposed surface of the ball relatively to its volume the less will be the oxidation of the metal in the ball after its separation from the excess slag. Consequently it is important to definitely limit the respective dimensions of the ball so that its shape will as nearly as practicable approximate the desired shape as above explained.

I have found that for best practice the depth of the ball formed in the slag receptacle should closely approach or approximate the depth of the slag before any of the molten refined ferrous material is poured in. However, the slag depth is also directly related to the temperature of the molten refined ferrous material as the hotter the molten refined ferrous material the deeper must be the slag (for a given temperature of the slag) in order to insure proper disintegration and welding of the metal in forming the ball. I have found that to avoid increasing the slag depth above that which is desired for formation of a ball of the preferred shape the temperature of the molten refined ferrous material as poured into the slag should be between about 2800° F. and about 2900° F.

Another and an important factor, however, is the temperature of the slag itself before the molten refined ferrous material is poured in. If the slag is relatively hot it will have to be relatively deep to accomplish the desired results in ball formation just as the slag would have to be relatively deep if the metal were relatively hot. On the other hand, if the slag is relatively cold the result may be a failure to properly disintegrate the metal and cause it to weld into the ball as the entrained slag would not have sufficient fluidity. I have found that the temperature of the slag should be between about 2475° F. and

about 2550° F. in order to form a ball of the desired shape when using molten refined ferrous material whose temperature as poured into the slag is between about 2800° F. and about 2900° F.

When the temperature of the slag in the bath is between about 2475° F. and about 2550° F. and the temperature of the molten refined ferrous material as poured into the slag is between about 2800° F. and about 2900° F. and the ball formed is of such shape that its greatest transverse dimension is not greater than twice its thickness the ball thus formed will be at optimum temperature and in optimum condition for the expelling of a maximum amount of slag in the press, resulting in the formation of wrought iron of superior quality. Under certain circumstances one or more of the factors above discussed may vary somewhat from the particular range specified and satisfactory results will be obtained, although in order to insure uniformly satisfactory results it is desirable to keep all of the factors simultaneously within the ranges stated.

Another advantage in making a ball whose greatest transverse dimension is not greater than twice its thickness is that such a ball may most efficiently be compressed or squeezed in the press. If a decidedly elongated ball or sausage-like wrought iron sponge mass is formed it is not only subject to excessive cooling and oxidation but is not susceptible of most efficient formation into a bloom or working mass in the press. Formerly when the rotary squeezer was used for squeezing out the excess slag it was thought by some to be desirable to form a substantially elongated ball, but such ball had disadvantages in respect of heat dissipation and oxidation and with the hydraulic press which is now preferred the ball is desirably of roughly spherical or cubical shape.

Since the volume of slag employed is several times the volume of metal (ordinarily between 8 and 20 times), the temperature of the slag is perhaps the most important factor in bringing about the desired results in the press and the production of wrought iron of superior quality. I have found that if the temperature of the slag before pouring in the molten refined ferrous material is maintained between about 2475° F. and about 2550° F. highly satisfactory results are obtained. This may at times be true even though the temperature of the metal may be somewhat outside the range above referred to and even though the shape of the ball may differ somewhat from the desired shape. However, as above indicated, when all of the factors mentioned are

kept within the limits herein defined uniform production of wrought iron of the highest quality is insured.

While I have described a present preferred method of practicing the invention it is to be distinctly understood that the invention is not limited thereto but may be otherwise variously practiced within the scope of the following claims.

I claim:

10. 1. In the manufacture of wrought iron by the Aston process, admixing molten refined ferrous material and molten slag having a temperature between about 2475° F. and about 2550° F. to form a wrought iron sponge ball, expelling a portion of the slag from the ball and working the wrought iron thus produced.
15. 2. In the manufacture of wrought iron by the Aston process, admixing molten refined ferrous material and molten slag having a temperature between about 2475° F. and about 2550° F. to form a wrought iron sponge ball whose greatest transverse dimension is not greater than twice its thickness, expelling a portion of the slag from the ball and working the wrought iron thus produced.
20. 3. In the manufacture of wrought iron by the Aston process, admixing molten refined ferrous material having a temperature between about 2800° F. and about 2900° F. and molten slag having a temperature between about 2475° F. and about 2550° F. to form a wrought iron sponge ball, expelling a portion of the slag from the ball and working the wrought iron thus produced.
25. 4. In the manufacture of wrought iron by the Aston process, admixing molten refined ferrous material having a temperature between about 2800° F. and about 2900° F. and molten slag to form a wrought iron sponge ball whose greatest transverse dimension is not greater than twice its thickness, expelling a portion of the slag from the ball and working the wrought iron thus produced.
30. 5. In the manufacture of wrought iron by the Aston process, admixing molten refined ferrous material having a temperature between about 2800° F. and about 2900° F. and molten slag having a temperature between about 2475° F. and about 2550° F. to form a wrought iron sponge ball whose greatest transverse dimension is not greater than twice its thickness, expelling a portion of the slag from the ball and working the wrought iron thus produced.
35. 6. In the manufacture of wrought iron by the Aston process, admixing molten refined ferrous material having a temperature between about 2800° F. and about 2900° F. and molten slag to form a wrought iron sponge ball whose greatest transverse dimension is not greater than twice its thickness, expelling a portion of the slag from the ball and working the wrought iron thus produced.
40. 7. In the manufacture of wrought iron by the Aston process, admixing molten refined ferrous material having a temperature between about 2800° F. and about 2900° F. and molten slag having a temperature between about 2475° F. and about 2550° F. to form a wrought iron sponge ball whose greatest transverse dimension is not greater than twice its thickness, expelling a portion of the slag from the ball and working the wrought iron thus produced.
45. 8. In the manufacture of wrought iron by the Aston process, admixing molten refined ferrous material having a temperature between about 2800° F. and about 2900° F. and molten slag having a temperature between about 2475° F. and about 2550° F. to form a wrought iron sponge ball whose greatest transverse dimension is not greater than twice its thickness, expelling a portion of the slag from the ball and working the wrought iron thus produced.

EDWARD B. STORY.